

June 17, 1952

L. F. REINARTZ ET AL

**2,600,575**

## TREATMENT OF MOLTEN METAL

Filed March 17, 1945

Fig. 1



Fig. 2



INVENTORS.  
BY Leo. F. Reinerz, and  
Charles R. FouleBessin  
Allen & Allen  
ATTORNEYS.

## UNITED STATES PATENT OFFICE

2,600,575

## TREATMENT OF MOLTEN METAL

Leo F. Reinartz and Charles R. Fon Dersmith,  
Middletown, Ohio, assignors to Armco Steel  
Corporation, a corporation of Ohio

Application March 17, 1945, Serial No. 583,350

3 Claims. (Cl. 75—56)

1

This application is a continuation in part of our copending application of the same title, Serial No. 393,424 filed May 14, 1941, now abandoned.

It has been understood that where molten metal is to be introduced into an open hearth furnace or equivalent refining device, theoretical advantages could be obtained by pretreating the molten metal with mill scale or other forms of iron oxide. These advantages include an immediate and valuable reduction in the silicon and manganese contents of the molten metal and, under some circumstances, reductions in the content of phosphorus, sulphur, and other impurities. The use of mill scale or other waste oxides would be valuable from the standpoint of utilization of waste materials; and a successful treatment would result in the realization of iron values from such materials.

Hitherto, in all attempts to treat molten blast furnace metal with iron oxide, the oxide was either added to the ladle in which the pig metal is tapped, or to the molten metal as it flows through the blast furnace runner, so that it will be carried by the metal into the ladle, or both; but the known procedures involve such serious difficulties that in all instances in which they have been tried, they have had to be abandoned.

The reaction between the metal and the oxide is exothermic and may become violent and explosive, so that the danger to workmen is excessive.

The preferred way of getting metal from the blast furnace to the open hearth is to collect the metal from the blast furnace runner in mixer cars, e. g. Pugh ladles, whence it is poured as required into open hearth ladles for charging. The Pugh ladles make the use of mixers unnecessary, and permit the holding of metal in molten form for as long as may be necessary.

But when iron oxide is added to the blast furnace metal as described, it can no longer be collected in a Pugh ladle. The reaction produces an acid slag of high melting point which builds up in Pugh ladles, attacking their linings and ultimately rendering them useless. Hence the metal must first be run and treated in an open top blast furnace ladle, from which, when the reaction is completed, it must be tapped into a Pugh ladle with removal of the slag. This involves extra equipment, labor and time delay, as well as substantial heat loss in the metal.

The treatment as hitherto known was incapable of chemical control. There is no way of ascertaining exactly the chemical content of a

2

batch of blast furnace metal in advance of tapping the furnace; but once the furnace is tapped, it is necessary to take the metal. Hence if it is to be treated with iron oxide, the oxide must be added by judgment or guess based upon observation of the action of the furnace.

10 The chief objects of our invention are the provision of a treatment method and apparatus whereby these disadvantages are all eliminated, and whereby the theoretical advantages of a pre-purification of the metal with iron oxide can be attained in practice.

15 It is an object of our invention to avoid the safety hazards involved in the former known treatment.

20 It is an object of our invention to provide a process in which blast furnace metal can be collected, handled, held and dispensed to the open hearth furnaces in the manner and by the means heretofore found most advantageous, but in which the metal may nevertheless be treated with iron oxide.

25 It is an object of our invention to provide a process of treating molten blast furnace metal with iron oxide in which any re-ladling for slagging purposes is eliminated entirely.

30 It is an object of our invention to provide a process of treating molten blast furnace metal with iron oxide in accordance with the principles of exact chemical control, and based upon the known content of the metal of the impurities to be removed.

35 It is an object of our invention to provide a process of treating molten blast furnace metal with iron oxide which requires no containers for molten metal other than those customarily used for untreated metal and which requires additional apparatus of negligible cost only.

40 We accomplish these objects, and others which will be pointed out herein or will be apparent to one skilled in the art upon reading this specification, by that certain construction and arrangement of parts and in that procedure, of which we shall now describe an exemplary embodiment.

45 Reference is made to the drawings wherein:

Figure 1 is a plan view of an exemplary treatment apparatus according to our invention.

Figure 2 is a side elevation thereof.

50 Our invention is based upon a concept of treating the molten metal very rapidly and in the increments desired for charging into the open hearth furnace, as against treating the whole molten metal content of a blast furnace cast as the metal is being tapped therefrom. In this fashion control may be exercised as hereinafter

explained, and the disadvantages of former procedures eliminated. But the successful operation necessitates carrying on the reaction not only in a controlled manner, but so rapidly as to bring it to completion within the space of time required for the filling of a vessel suitable for charging an open hearth furnace. We have found that this may be accomplished by special procedures in carrying on the reaction, and under the special circumstances hereinafter outlined.

We shall use the term "blast furnace" to indicate generally the point of origin of the molten metal; and we shall use the term "open hearth furnace" as indicative of the means for refining the molten metal.

In our practice the pig metal from the blast furnace is tapped therefrom and run into mixer cars or Pugh ladles, as in the accepted practice for non-treated metal. In these ladles the molten metal can be held without losing its molten character for such periods of time as to permit convenient charging of the open hearth furnaces in accordance with their requirements. No attempt is made at this stage to treat the metal; but during the holding period an analysis is made of the metal to determine its content of impurities, e. g. of silicon and manganese. On this analysis a calculation is made of the quantity of iron oxide required per unit quantity of the molten metal to reduce its content of impurities to a desired value in the light of advantageous open hearth practice.

In ordinary practice for charging the open hearth furnaces, the metal is poured as required from the Pugh ladle into open hearth ladles. The apparatus departure we make in accordance with this invention involves the provision of a runner to receive the metal from the Pugh ladle and deliver it to the open hearth ladle, together with a means for feeding iron oxide into the runner.

The molten metal is poured into the runner under conditions in which the volume of the stream can be controlled. Increments of oxide are introduced into the runner along with the molten metal. The increments so added total the quantity of iron oxide shown to be required by the analysis for the particular quantity of metal to be poured through the runner into the desired batch receiving vessel.

The molten metal, having been treated with the iron oxide is delivered at the end of the runner into a ladle suitable for charging the metal into the open hearth. The pouring is discontinued as soon as the desired quantity of metal has been introduced into the ladle. The process does not delay the transfer of the metal from the Pugh ladle to the furnace.

It will now be evident that the success of our process involves carrying on the reaction in a very rapid and controlled manner so that it will be completed or substantially completed during the short time required to fill an open hearth ladle from a Pugh ladle (or as hereinafter set forth, from two Pugh ladles pouring simultaneously and rapidly). We have found that this can be done if the following conditions are met:

1. It is essential not only that the iron oxide be added to the molten metal in the runner but also that it be mixed with the molten metal in the runner. If iron oxide be added to molten metal in a blast furnace runner it tends to float upon the surface of the metal and is carried thereby into the ladle. In this event, as also in

the case where the oxide is added directly to the ladle, whatever mixing there is occurs primarily in the ladle. This will not serve our purpose; and we can neither add all our oxide to the ladle nor can we allow it to be floated into the ladle substantially unmixed. In either event the reaction is incomplete and uncontrollable.

2. We provide a runner so constructed as to have an enfolding function for the iron oxide. Our runner has a receiving head or hopper into which we pour the metal in one or more streams and into which we also introduce the oxide. Mixing occurs at this point. Again the open runner leading from this head or hopper is not straight but is tortuous in the sense that it has one or more sharp bends at which straight sections join each other at substantial angles in connecting boxes. Thus the direction of flow of the metal is sharply changed, and at the boxes the metal rides up the sides at the outside of the turns and, as it were, folds over upon itself, enclosing and enveloping any quantities of the oxide which tend to float on top, and actively mixing the oxide with the metal before the metal enters the ladle.

3. The iron oxide must be added gradually and substantially uniformly to the molten metal. This is done by a mechanically actuated feed hopper located above the receiving head. During the greater portion of the pouring, and preferably during all of it, equal increments of the oxide are added to equal increments of the molten metal. The metal is poured rapidly from one or two Pugh ladles into the receiving head or hopper of the runner, but evenly, and the oxide is thus evenly and fairly uniformly associated with the metal, quantity for quantity, before the metal enters the open hearth ladle. The rate of pour from the Pugh ladle or ladles is of course controlled by the motors tilting the ladles, and the rate of feeding of the oxide is controlled by a motor on or in connection with the oxide hopper.

4. Nevertheless, the type of treatment reagent must be one very rapid in its action. Not every form of iron oxide can be used. Iron ores of various types, oxide bearing flue dusts and the like, available in the former processes, are not sufficiently rapid nor sufficiently easily miscible with the molten metal for our procedure. We have found that mill scale is, however, sufficiently active and sufficiently heavy to enable us to treat metal in the way herein described, and this is the oxide which we use.

When these conditions are met, the reaction takes place in substantial measure in the runner and also continues for a short period in the ladle. It is strongly exothermic and very active. The metal in the runner gives off a shower of sparks, but there is little likelihood of explosion if precautions are taken to assure a dry condition of the mill scale. The reaction is largely controlled by the continuous proportioning of the mill scale to the molten metal. The circumstances are such that the operators may be adequately shielded and protected. They are not required to work in exposed positions about an open runner as at the blast furnace. The flow of metal from the Pugh ladles may, of course, be cut off at any time.

5. The metal collecting in the open hearth ladle is also active, but less violently so. If, as the ladle becomes nearly full, a tendency to boil over appears, the metal may be quieted by the addition of a smaller quantity of salt to the ladle. This is not usually necessary; the reaction rapidly

spends itself, and the high-melting point acid slag formed by the reaction begins to congeal on the top of the molten metal.

The ladle is then carried directly to the open hearth and the hot metal charged into it. This may, if desired, be done by tapping the ladle so as to separate the slag. In the majority of instances nearly all the slag will have formed a stiff crust on the metal, so that it is possible to pour the metal from the ladle into the open hearth by tilting the ladle in the usual way, the bulk of slag remaining in the ladle. Afterward the slag may be removed from the ladle by up-ending it over a thimble or the like.

Since the metal is treated as desired for charging, and since the treated metal is charged at once into the open hearth without re-ladling for slag removal, the heat generated by the exothermic reaction is no longer lost; but the charged metal is hotter than the metal in the Pugh ladles. This is not only important in the matter of open hearth efficiency, but is especially valuable when it has been necessary for any reason to hold the metal in the Pugh ladles until its temperature has become too low.

The distance of the blast furnace from the open hearth is not in any sense determinative of the utility of our process. The Pugh ladle, as in ordinary practice, permits holding the molten metal until required for charging, and also permits its interim transportation should that be necessary. For reasons which will now be clear, however, our treatment of the molten metal with mill scale, to realize all of its advantages, must be carried on so close to the open hearth that the treated metal may be collected in an open hearth charging ladle and charged directly into the furnace.

All of these factors permit us to introduce into our open hearth furnaces charges of molten metal of enhanced iron value and at higher temperatures than would be possible otherwise. There molten metal charges, together with charges of scrap and the like, and charges of treatment reagents, permit us to operate the open hearth furnaces under improved conditions. The treated metal may be introduced without that slag which results from the treatment with the mill scale. The added heat enables us to shorten the cycles in the open hearth furnace, and the pre-reduction of the silicon and manganese contents of the molten metal reduces the slagging problem in the furnace.

In the drawings of our exemplary apparatus, we have indicated at 1 a framework or housing, and at 2 and 3 mixer cars of the Pugh type. These cars move on tracks 4 and 5 at a high level on the framework and interspaced, so that the mixers of one or both mixer cars may be simultaneously rotated on their axes to pour the molten metal into the head 6 of the runner which is located between the two tracks. The hopper for the mill scale is indicated at 8. This hopper is mechanically actuated to deliver a controlled stream or controlled increments of the mill scale into the head of the runner, as required by a controlled rate of pour from the Pugh cars.

The runner proper is a refractory lined structure of tortuous character to assist in the mixing and comprises angularly related straight sections 7 and corner boxes 7a wherein the over-folding action of the molten metal takes place. It may also have, if desired, one or more vertical drops in it to enhance the mixing action. It is located between the tracks and at a lower level in

the framework 1 as shown. This permits us to fence or house the runner, as indicated at 9, 10 and 11, whereby the workmen are protected from the violence of the reaction occurring therein.

5 The operator who controls the rate of pouring of the hot metal and the addition of the scale may be conveniently and safely located in a control house provided with a safety glass window located immediately behind and below the scale hopper. The runner, near the end remote from the head, passes under one of the tracks as shown and delivers the molten metal into a ladle 12 located at a still lower level. When the ladle is full or has received the total quantity of molten metal intended for it, it is picked up by a crane and tapped or poured into the open hearth furnace or furnaces (not shown).

It will have been noted that we preferably provide two tracks and two mixer cars for reasons 20 already given. But we may thus, if desired, pour metals of dissimilar analyses simultaneously into the runner for treatment. This practice improves uniformity of the addition of hot metal in the open hearth practice, and enables us to make

25 minimum additions of scale in our treatment. In regular practice, by mixing metal from two ladles, or by pouring single ladles, as the analysis may indicate, we are enabled to work closer to a common end point, say 0.35 to 0.45% silicon, 30 which will allow the use of a maximum ratio of hot metal to scrap in the open hearth, without charge ore additions or permit a still higher hot metal ratio with only small charge ore additions. Charge ore additions are likely to cause serious foaming of the metal bath in the open hearth furnace. We secure a greater uniformity of our metal because of close control of the silicon in the hot metal, in addition to the other advantages of our process.

40 It is not outside the purview of our invention to use other treatment reagents along with mill scale for special purposes. In some operations, finely crushed manganese ore may be used like mill scale to reduce silicon, while preserving manganese in the molten metal. Manganese ore likewise has an exothermic reaction with molten iron.

Other treatment agents may also be employed. Soda ash, barium oxide or other alkali compounds 50 may be added to reduce sulphur. These do not have a significant exothermic effect, but may be added along with mill scale or manganese ore. The very corrosive slag they produce can, in our process, be kept out of the open hearth furnace or other refining means.

Modifications may be made in our invention without departing from the spirit of it. Having thus described our invention, what we claim as new and desire to secure as Letters Patent is:

60 1. Apparatus for the treatment of molten pig iron metal comprising interspaced tracks upon which carriers for molten metal may be run, means for supporting said tracks at an elevated level, a runner located between said tracks, 65 adapted to receive molten metal from said carriers simultaneously and located at a lower level, a hopper adapted to deliver mill scale into said runner, and a ladle located at a still lower level, and housing means surrounding said runner.

70 2. Apparatus as claimed in claim 1 in which said ladle is located at the side of one of said tracks remote from the interspace between the said tracks, and wherein an end of said runner passes through one of said housing means.

75 3. A process of supplying improved molten

blast furnace iron to an open hearth furnace, which comprises tapping the molten metal from the blast furnace into a refractory lined vessel, and at a point adjacent an open hearth furnace, pouring it rapidly from said vessel into a tortuous runner, adding mill scale to it in the said runner in increments proportioned to the rate of flow therethrough, adding equal increments of mill scale to the runner along with equal increments of molten metal during a portion at least of the pouring, the mill scale mixed with the molten metal being proportioned to the known content of silicon and manganese in the molten metal, the molten metal poured into the runner being simultaneously derived from sources of different analyses, delivering it from the runner into a ladle in quantity suitable for charging it into the open hearth, discontinuing the said pouring upon the accumulation of a charge in said ladle, and promptly transferring the metal from said ladle into said open hearth furnace.

LEO F. REINARTZ.  
CHARLES R. FON DERSMITH.

## REFERENCES CITED

The following references are of record in the file of this patent:

## UNITED STATES PATENTS

| Number    | Name     | Date          |
|-----------|----------|---------------|
| 843,582   | Campbell | Feb. 12, 1907 |
| 874,391   | Chute    | Dec. 24, 1907 |
| 1,863,686 | Corsalli | June 21, 1932 |
| 2,302,999 | O'Brien  | Nov. 24, 1942 |

## FOREIGN PATENTS

| Number | Country       | Date    |
|--------|---------------|---------|
| 16,601 | Great Britain | of 1911 |

## OTHER REFERENCES

Blast Furnace Practice, pages 40 to 45, and 275. Edited by Sweetser. Published in 1938 by the McGraw-Hill Book Company, New York.

Open Hearth Proceedings, A. I. M. E., 1940, page 141. Published by the American Institute of Mining and Metallurgical Engineers, New York.

Open Hearth Proceedings, A. I. M. E., 1941, page 141.